

## UNITED STATES PATENT OFFICE

2,563,431

METHOD OF IMPROVING THE RESISTANCE  
TO CORROSION AND ABRASION OF CERTAIN COATED ALUMINUM SURFACESFrank Palin Spruance, Jr., Ambler, Pa., assignor  
to American Chemical Paint Company, Ambler,  
Pa., a corporation of DelawareNo Drawing. Application September 20, 1949,  
Serial No. 116,858

2 Claims. (Cl. 148—6.16)

1

This invention relates to the art of coating aluminum and alloys thereof in which aluminum is the principal ingredient and in the following disclosure, as well as in the appended claims, the word "aluminum" is intended to be understood as including alloys thereof in which aluminum is the principal or dominant ingredient.

It has been known to those skilled in this art that aluminum surfaces can be improved as to their corrosion resistance and paint holding ability if they are coated by subjecting them to the action of an acid aqueous solution, the essential coating-producing ingredients of which are fluoride ions, dichromate ions and ions from the class of acids consisting of phosphoric and arsenic acids. Coating treatments of this kind are fully described and claimed in my prior U. S. patents, No. 2,438,877 issued March 30, 1948, and No. 2,471,909 issued April 5, 1949, as well as in my copending application No. 38,192 filed on July 12, 1948, now U. S. Patent No. 2,494,910. Another treatment of this nature is disclosed in the U. S. Patent No. 2,472,864 issued on June 14, 1949, to James H. Thirsk and myself. In the several disclosures just mentioned, various methods and materials are described for the coating of aluminum by treating it with acid aqueous solutions of the nature above specified.

The present invention is based upon the discovery that aluminum surfaces which are coated in accordance with the teachings of the foregoing patents and application may have their resistance to corrosion and abrasion substantially improved if the coated surfaces are subsequently treated with certain aqueous solutions to be described below and the principal object of the present invention is to so improve such coated aluminum surfaces. Another important object is to provide a method for treating such coated aluminum surfaces which will permit a much greater tolerance to wider variations in the coating solutions heretofore familiar to those skilled in the art—for example, those disclosed in the above referred to patents and application. A concomitant object of the present invention is to make it possible to practice the prior coating procedures with somewhat less exactitude and care, and therefore with less experienced personnel which, of course, results in a corresponding decrease in the costs of the coating operation. The present invention also has for an object the provision of a method which minimizes the tendency to powder, which has heretofore been characteristic of some of the coatings produced by prior procedures unless the processes are op-

2

erated with a great deal of care and exactitude.

By way of examples of coatings produced by previous methods upon which coatings my present invention is particularly useful, I wish to cite the following. For instance, a coating may be produced by means of a solution which is formulated in accordance with

## Formula I

|                                  | Grams |
|----------------------------------|-------|
| 10 Sodium fluoride               | 5     |
| Chromic acid (CrO <sub>3</sub> ) | 10    |
| Phosphoric acid, 75%             | 64    |
| Water, to make 1 liter.          |       |

15 A coating may be obtained by immersing the aluminum surface in the foregoing solution or by flowing or spraying the solution upon the work or by any other convenient technique familiar to the art. Of course, the solution must be left in contact with the metal long enough to act thereupon until the coating is produced. The time required to produce the coating will vary, of course, with the temperature and method of applying the solution to the metal. At ordinary living temperatures it may require as much as five to ten minutes to produce an appreciable coating with the above solution when the solution is flowed upon the metal but this time can be substantially reduced, say to as little as one to two minutes or even less by suitably heating the solution and using it in a spray process.

Other representative formulae for various coating solutions of the nature disclosed in the above referred to patents and application are as follows:

## Formula II

|                               | Grams |
|-------------------------------|-------|
| Ammonium acid difluoride      | 30    |
| Potassium dichromate          | 20    |
| Ammonium dihydrogen phosphate | 80    |
| Water, to make 1 liter.       |       |

## Formula III

|                                  | Grams |
|----------------------------------|-------|
| Sodium fluoride                  | 5     |
| Chromic acid (CrO <sub>3</sub> ) | 10    |
| Phosphoric acid, 75%             | 61    |
| Arsenic acid                     | 2     |
| Water, to make 1 liter.          |       |

## Formula IV

|                                  | Grams |
|----------------------------------|-------|
| Sodium fluoride                  | 5.0   |
| Chromic acid (CrO <sub>3</sub> ) | 10.0  |
| Arsenic acid                     | 92.5  |
| Water, to make 1 liter.          |       |

After treatment with any of the typical solu-

tions described above or with other coating solutions of a similar nature, the essential coating-producing ingredients of which are fluoride ions, dichromate ions and ions from the class of acids consisting of phosphoric and arsenic acids, the coated surface may be rinsed with water and then treated in accordance with the present invention, or the method of the present invention may be applied without a prior rinse with water. The solutions used in carrying out the present invention may be applied by dipping the work into the solution or by spraying or flowing the solution over the surface or by means of any other convenient technique in which the solution can be brought into contact with the coated surface. The length of time in which the coated metal surfaces are in contact with the solution is not critical, and, in fact, may be rather brief, say 20 to 30 seconds or so. Also the temperature of the solution is not critical, although it is better not to use a solution which is hotter than 140° F. and I prefer to use it at approximately 120° F., or lower. After removal from the solution, drying of the surface completes the treatment whether or not preceded by water rinse.

The treatment of the present method makes use of a relatively strong solution of water soluble dichromate or dichromates taken from the class which consists of the alkali-metal dichromates and ammonium dichromate. The concentration of the dichromate ions ( $Cr_2O_7$ ) should lie between 3.5 and 45 grams per liter at a pH of from 5.0 to 6.5. Typical examples of said soluble dichromates are sodium dichromate and ammonium dichromate, and the following are illustrative formulae for such treating solutions:

*Formula V*

Ammonium dichromate, 20 grams  
Water, to make 1 liter.

*Formula VI*

Sodium dichromate, 30 grams  
Water, to make 1 liter.

In the two formulae just given, the water is 45 ordinary tap water, containing the customary salts. Had the water used been distilled or deionized, the pH would have been low and would have to be adjusted by addition of a caustic. In some localities the pH of the raw water may be 50 high enough to warrant the addition of an acid to bring the pH within the operating range. However, when the treating solution is in the operating range of 5.0 to 6.5 there are enough

buffer salts present to discourage any marked fluctuations of pH as work is being treated.

The use of such treating solutions as just described imparts to the coated surface quite a high degree of corrosion resistance and also tends to remove any of the powder which may have been formed on the coated surface by the coating solutions typified by Formulae I to IV.

It should be noted that if the concentrations 10 of the treating solutions go over the maximum shown above that there is a tendency for the treatment to dissolve the coating while, on the other hand, when the concentrations fall below 3.5 grams per liter soluble dichromate expressed 15 as  $Cr_2O_7$ , the beneficial effects are greatly diminished.

This application is a continuation-in-part of my earlier application Serial No. 90,562, filed April 29, 1949, now abandoned.

20 I claim:

1. In the art of coating aluminum to increase its resistance to corrosion and abrasion where the surface of the metal is coated by subjecting it to the action of an acid aqueous solution the 25 essential coating-producing ingredients of which are fluoride ions, dichromate ions and ions from the class of acids consisting of phosphoric and arsenic acids; the method which consists in treating a surface so coated with an aqueous solution 30 having a pH of from 5.0 to 6.5 and containing as its essential active ingredient a water soluble dichromate taken from the class which consists of the alkali-metal dichromates and ammonium dichromate in a concentration expressed as  $Cr_2O_7$  35 of from 3.5 to 45 grams per liter.

2. The method according to claim 1 in which the treating solution is maintained at a temperature not to exceed approximately 140° F.

FRANK PALIN SPRUANCE, JR.

40

REFERENCES CITED

The following references are of record in the file of this patent:

UNITED STATES PATENTS

| Number    | Name                  | Date          |
|-----------|-----------------------|---------------|
| 1,946,151 | Edwards               | Feb. 6, 1934  |
| 2,213,263 | Thompson et al.       | Sept. 3, 1940 |
| 2,245,609 | Romig                 | June 17, 1941 |
| 2,312,855 | Thompson              | Mar. 2, 1943  |
| 2,314,887 | Lodeesen              | Mar. 30, 1943 |
| 2,318,656 | Thompson              | May 11, 1943  |
| 2,472,864 | Spruance, Jr., et al. | June 14, 1949 |